

75-232

SR

XR 2,302,615

TOSS Reference

Search Room

Patented Nov. 17 1943

TX 75-232

2,302,615

## UNITED STATES PATENT OFFICE

2,302,615

## BRIQUETTE FOR THE ADDITION OF MOLYBDENUM TO FERROUS ALLOYS

Arthur Linz, New York, N. Y., assignor to Climax Molybdenum Company, New York, N. Y., a corporation of Delaware

No Drawing. Application April 22, 1941, Serial No. 389,751.

(Cl. 75—133)

7 Claims.

The present invention relates to a novel and improved molybdenum addition agent for the production of ferrous alloys.

Objects and advantages of the invention will be set forth in part hereinafter and in part will be obvious herefrom; or may be learned by practice with the invention, the same being realized and attained by means of the compositions, steps, processes and instrumentalities pointed out in the appended claims.

The invention consists in the novel compositions, steps, processes, combinations and improvements herein shown and described.

The present invention has for its object the provision of a novel and improved molybdenum containing alloying agent which is of wide usefulness in the production of molybdenum containing ferrous alloys. The invention further provides a novel and improved molybdenum briquette which can be economically produced and contains a minimum of foreign material. The invention has for another object the provision of an improved molybdenum containing briquette which can be used in practically all ways that other molybdenum addition agents have heretofore been used, and which is superior in one respect or another to all of the previous molybdenum addition agents.

Heretofore molybdenum has been added to ferrous alloys, by a large number of different processes involving a wide variety of different addition agents. Molybdenum sulfide or molybdenite concentrates have been proposed and used as an addition agent but have proved to be of very limited application due to the relatively large proportion of sulphur contained therein and introduced thereby into the ferrous alloy. Molybdenum trioxide, roasted molybdenite and molybdenum dioxide, all oxides of molybdenum, have been used as addition agents, but their use has almost invariably been attended by excessive loss of molybdenum, resulting in an increased cost of producing the alloy, and furthermore their use has been limited to the production of ferrous alloys to contain less than 1 per cent of molybdenum. Calcium molybdate, combinations of lime with lower oxides of molybdenum and mechanical mixtures of calcium oxide and molybdenum trioxide have also been used as addition agents, but their use is limited to the production of iron-molybdenum alloys containing less than 1 per cent of molybdenum, and have been attended by an unavoidable increase in the slag, as well as by the detrimental inclusion of slag within the alloy.

Various varieties of ferro-molybdenum have also been widely used for the production of molybdenum-bearing ferrous alloys, and while there is no practical limit to the amount of molybdenum which may be contained in the alloys produced therewith, this type of addition agent has necessarily increased the cost due to the extra operations required for the manufacture of ferro-molybdenum. Ferro-molybdenum has the added disadvantage that it sinks to the bottom of the ladle and the resulting ferrous alloy is rendered homogeneous only with difficulty. Briquettes of a molybdenum oxide with carbon have been widely used, and while they avoid many of the disadvantages of the other alloying agents, they produce a boil, and when large percentages of molybdenum are to be added in this way, the gas evolution may be excessive. Molybdenum silicide has also been used as an addition agent where a fairly high silicon content in the resulting alloy is unobjectionable. At other times, pure molybdenum powder has been used as the addition agent, but aside from the relatively expensive cost of producing molybdenum powder, the absorption of the molybdenum into the ferrous alloy is too slow to be commercially desirable.

In general, the various ways in which molybdenum has been added to ferrous alloys have been less effective substitutes for the universally useable ferro-molybdenum, which has its relatively high cost and its relatively high specific gravity as its primary commercial disadvantages.

In addition to the foregoing, there have been other minor ways proposed for the addition of molybdenum to ferrous alloys, but these have not met with any considerable commercial use, and among them may be mentioned the mixtures of molybdenum trioxides with silicon and/or ferro-silicon.

The present invention provides an economical molybdenum addition agent for ferrous alloys, which eliminates the use of any relatively expensive reducing agents, the availability of which may be restricted, such as aluminium, silicon, magnesium and calcium, requires a minimum of equipment for its production, eliminates the objections which have existed with respect to all of the commercially used addition agents set forth above, and does not result in the introduction into the molten ferrous metal of any foreign material.

Thus, the molybdenum addition agent of the present invention provides a universally acceptable molybdenum containing compound for the introduction of molybdenum into ferrous alloys

which can be used, with considerable savings, as a substitute for any of the molybdenum addition agents heretofore found useful, thereby simplifying the production of molybdenum addition agents in general, as well as reducing the variety of such addition agents which must be carried on hand by the manufacturer or steel maker.

In accordance with the present invention, roasted molybdenite concentrates are partially reduced to form crude molybdenum oxides or crude molybdenum metal powder containing some of the molybdenum oxides as impurities, and this reduced roasted concentrate is mixed intimately with relatively fine powdered, granular or flakelike iron. The resultant intimate mechanical mixture of these substances is highly compressed to form briquettes which are preferably of uniform size. Due to the peculiar characteristics of the molybdenum compound and the iron particles, no foreign binder is needed for the coherence of this mixture, and the briquettes preferably contain not more than a trace of carbon or other impurities.

It will be understood that the foregoing general description and the following detailed description as well are exemplary and explanatory of the invention but are not restrictive thereof.

Referring now in detail to the present preferred and illustrative embodiments of the invention, the novel and improved molybdenum containing briquettes are formed from partially reduced roasted molybdenite concentrates which are a crude form of molybdenum trioxide. The roasted concentrates are reduced with carbonaceous material in a beehive or coke oven, and the reduction is carried on until the oxide contains from 50 to 60 per cent molybdenum dioxide, from 20 to 30 per cent of molybdenum oxide, while the remainder is metallic molybdenum and gangue; or, the reduction may be carried on still further until the molybdenum is present as from 50 to 60 per cent metallic molybdenum, 20 to 30 per cent molybdenum oxide, and the balance molybdenum dioxide and gangue. The reducing agent may conveniently be carbon or some other reducing agent such as pitch which is substantially entirely removed from the molybdenum compound by the end of the reduction process. Preferably, not more than 0.25% carbon is contained in the briquettes as they are finally made up. Thus, the reduced molybdenite concentrates contain from approximately 7.5% to 17% oxygen, while the crude metallic molybdenum or highly reduced molybdenum oxides contain from about 7.5% to 11% oxygen, as contrasted with the 25% oxygen content of molybdenum dioxide and the 33% oxygen content of molybdenum trioxide.

The reduced roasted concentrates are generally in the form of relatively small particles, the individual particles or grains having a center which is largely molybdenum dioxide surrounded by a considerable layer of molybdenum monoxide, which in turn is coated with powdered metallic molybdenum, these successive layers gradually merging into each other and being formed as the result of a more intensive reducing action on the surface of the particles.

The iron to be intimately mixed with the partially reduced molybdenum oxides may consist of powdered granular or flakelike iron containing the normal impurities, and even substantial amounts of iron oxide will not interfere with the results to be obtained.

Preferably the partially reduced roasted molybdenite concentrates are mixed with from 10 to 50

per cent of the iron particles, although as little as 5 per cent or as much as 70 per cent of the iron particles may be added to the reduced molybdenum compound. This mixture is thoroughly mixed until the molybdenum containing particles and the iron particles are intimately mixed, and the resulting mixture is briquetted to form relatively large briquettes which may conveniently contain a predetermined weight of metallic molybdenum. During the briquetting operation, the intimately mixed particles of the reduced molybdenum oxides and the iron particles are subjected to a relatively high pressure, and due to the different nature of the materials, the mixture is compressed into a relatively hard, coherent mass which can be shipped and will stand considerable rough handling without excessive crumbling.

In use, the briquettes may be treated in practically the same manner as is customary with ferro-molybdenum. They may be added to the steel furnace or ladle, and the molybdenum is rapidly absorbed by the melting or molten steel. Similarly, they may be added to the furnace or ladle during the manufacture of molybdenum containing cast iron. The briquettes sink just below the interface of the slag and molten metal, the slag protecting the metallic molybdenum from oxidation, at the same time that it allows it to be rapidly dissolved in the molten iron or steel. Inasmuch as the briquettes do not sink to the bottom of the ladle, the resulting alloy readily and quickly becomes homogeneous, and no difficulty is experienced through slow dispersion of the molybdenum throughout the alloy.

The briquettes contain no foreign material, no added impurities are introduced into the alloy, and due to the fact that the molybdenum is present in the briquettes in partly reduced form, the molybdenum is put into the steel or iron with almost an absolute minimum of chemical reaction, only ferro-molybdenum having less chemical reaction. Thus, the briquettes of the present invention can replace to advantage all of the molybdenum addition agents which have heretofore been used, with the added advantage that the briquettes of the present invention can be produced much more readily, and with less expense than any of the other molybdenum addition agents including ferro-molybdenum.

The invention in its broader aspects is not limited to the specific compositions, processes and steps described and departures may be made therefrom within the scope of the accompanying claims without departing from the principles of the invention and without sacrificing its chief advantages.

What I claim is:

1. A briquette for the addition of molybdenum to ferrous alloys consisting essentially of reduced molybdenum trioxide containing from approximately 7.5% to 17% oxygen and iron particles intimately mixed together.

2. A briquette for the addition of molybdenum to ferrous alloys consisting essentially of crude molybdenum powder containing from approximately 7.5% to 11% oxygen and iron particles intimately mixed together.

3. A briquette for the addition of molybdenum to ferrous alloys consisting substantially entirely of particles of reduced molybdenum trioxide the outer portions only of which are completely reduced molybdenum trioxide and particles of iron intimately mixed together and highly compressed to form a coherent mass.

4. A briquette for the addition of molybdenum

to ferrous alloys consisting substantially entirely of particles of highly reduced molybdenum tri-oxide containing less than 17% oxygen with the outer portions only substantially completely reduced to metallic molybdenum intimately mixed together and highly compressed to form a coherent mass. 5

5. A briquette for the addition of molybdenum to ferrous alloys consisting substantially entirely of particles of reduced molybdenum trioxide the outer portions only of which are completely reduced molybdenum trioxide and particles of iron intimately mixed together and highly compressed to form a coherent mass and containing less than 0.25% carbon. 10 15

6. A briquette for the addition of molybdenum to ferrous alloys consisting substantially of particles of reduced molybdenum trioxide the outer portions only of which are completely reduced molybdenum trioxide and from 5% to 70% particles of iron intimately mixed together and highly compressed to form a coherent mass.

7. A briquette for the addition of molybdenum to ferrous alloys consisting substantially of particles of reduced molybdenum trioxide the outer portions only of which are completely reduced molybdenum trioxide and from 10% to 50% particles of iron intimately mixed together and highly compressed to form a coherent mass.

ARTHUR LINZ.